

Patented May 21, 1929.

1,713,834

# UNITED STATES PATENT OFFICE.

HEINRICH KOPPERS, OF ESSEN-RUHR, GERMANY, ASSIGNOR TO THE KOPPERS DEVELOPMENT CORPORATION, OF PITTSBURGH, PENNSYLVANIA, A CORPORATION OF PENNSYLVANIA.

## HEATING SUBSTANCE SUSCEPTIBLE TO OXIDATION.

No Drawing. Application filed July 6, 1921, Serial No. 482,805, and in Germany May 13, 1928.

The invention relates to a process for heating or burning substances susceptible to oxidation, such as iron, steel, porcelain and the like; and has for its objects to prevent such oxidation and its deleterious consequences by maintaining a reducing atmosphere in direct environment of such substances by the intimate contact of the substances with carbon; also to do this without requiring a surplus amount of fuel gas and without requiring firing with an insufficient amount of air.

In heating, for instance iron and steel, and in burning, for instance porcelain, the prevention of oxidation plays an important part, be it to avoid losses by burning or an impairment of the quality of the iron or steel, or to obviate the discoloration of the porcelain. Oxidation in this connection not only is caused by the oxygen of the air but also by carbonic acid and steam. In the heating of iron and steel not only an attack on the iron itself is involved but also on the ingredients important to its quality, such as silicon, carbon and manganese. In the burning of porcelain this oxidizing effect shows itself in the form of a yellow coloring owing to the iron oxide which causes the final product to become spotted and discolored.

In order to avoid such oxidizing phenomena, it has been the practice heretofore to avoid a surplus of oxygen as much as possible during the heating; since an exact observance of the conditions necessary for complete combustion is, of course, a practical impossibility, it was always necessary to work with a corresponding lack of air or a gas surplus, which greatly impaired the economy of the firing plant, quite aside from other practical drawbacks. In burning porcelain, this so-called smoking fire makes itself felt by the heavy smoking of the chimneys, in which connection the sooty flame frequently shoots out of the chimney, thus also causing a pollution of the atmosphere and annoyance to the neighborhood.

According to the invention, in heating such substances susceptible to oxidation, a control of the heat with the maximum efficiency attainable in actual practice is rendered possible without an oxidation of the substances to be heated, annealed or burnt taking place, this result being accomplished

by maintaining in the direct vicinity of these substances a reducing atmosphere, for example by subjecting the respective substances, while in intimate contact with carbon, to the heating operation. In case this involves, for instance in pre-heating ovens for ingots and the like, objects which possess large dimensions and can also undergo separate treatment in other ways, said objects are coated with a protective layer of graphite and clay, while in connection with smaller objects, for instance rods which lie on the hearth body, the latter are covered with powdered graphite or comminuted carbon bricks; in place of the graphite it is also possible to use calcined coke, since carbon is converted, in the calcining of coke, into a not easily combustible form. A chemical action of the carbon on iron and steel is thereby practically precluded. The layer of coke powder can be so thick that the rods are in part embedded therein. This also replaces the heretofore customary covering of the hearth of such ovens with sand which fluxes with the resultant iron oxides and flows off as silicate.

In connection with the heating of pipe strips to welding heat before the tube rolls, where the welding and shaping take place at the same time, a considerable loss by oxidation is incurred to-day which has an unfavorable effect on the quality and production. By covering the oven hearth with calcined carbon, which has no carbonizing effect but only protects against oxidation, and by scattering said carbon over the pipe strips, the heavy losses by oxidation are prevented and the production and quality of the pipes are enhanced. The pipe strips brought to welding heat should remain in a reducing gas atmosphere from the welding ovens to the rolls, so that no roll scale or oxide may impair the welding.

The guiding idea can be realized in a highly advantageous manner in burning porcelain or any substances which it is customary to burn in capsules. Here, while operating the fire strictly according to economic viewpoints in every other respect, the reducing atmosphere necessary is produced within the capsules by adding to each capsule a certain quantity of carbon, for instance in the form of charcoal, which is made at the normal temperature, approximately 450 de-

degrees centigrade. This calcined carbon consumes the oxygen and takes care that a reducing atmosphere always prevails in the capsule. The amount of gas in the capsule 5 or glowing pot adjusts itself in equilibrium according to the temperature, with reference to the easily reacting carbon, in conformity with the proportions made known by Bou-douard,  $O_2:C:CO(CO_2)$ . The receptacles, 10 such as capsules or glowing pots, must be somewhat tightly sealed, in order that the oxidizing tuyère gases may not have free access to the material.

What is claimed is—

- 15 1. The process for heating or burning substances susceptible to oxidation, characterized by a reducing atmosphere being maintained, in direct environment of the bodies to be heated, by the intimate contact of these 20 substances with not easily combustible carbon, to prevent oxidation, without effecting carbonizing, of said substances and in order to make it possible to carry out the firing with the highest practical efficiency, without 25 requiring a fuel gas surplus and lack of sufficient air to support substantially complete combustion of such fuel gas.
2. The process according to claim 1, characterized by the substances to be heated, 30 being specially surrounded with a protective layer of graphite and clay.
3. The process according to claim 1, char-

acterized by the substances to be heated, being embedded in comminuted hard carbon distributed on the hearth of the oven, the 35 carbon being previously heated to such an extent that a chemical action of the carbon on the substances being subjected to heat treatment does not take place for all practical purposes.

40 4. The process according to claim 1 for heating rods in the manufacture of welded iron pipes and the like, characterized by heating the rods in a reducing gas atmosphere and maintaining the rods in the reducing gas atmosphere from the ovens to the rolls so that the welding may not be weakened by roller scale or oxide.

45 5. The process according to claim 1 for the heat treatment of substances in capsules, characterized by introducing at any time into the capsule a certain quantity of carbon, for instance charcoal made at the normal temperature, which prevents oxidation in 50 the capsule.

55 6. The herein described process for heating substances and protecting them against oxidation, which consists in maintaining calcined carbon about said substances while they are being heated to prevent oxidation, without effecting carbonizing, of said substances.

HEINRICH KOPPERS.